

Patented June 23, 1925.

1,542,965

# UNITED STATES PATENT OFFICE.

HELENA S. SADTLER, OF SPRINGFIELD TOWNSHIP, MONTGOMERY COUNTY, PENNSYLVANIA.

## INDELIBLE TRANSFER COMPOUND.

No Drawing.

Application filed July 14, 1923. Serial No. 651,622.

To all whom it may concern:

Be it known that I, HELENA S. SADTLER, a citizen of the United States, and a resident of Springfield Township, in the county of Montgomery and State of Pennsylvania, have invented an Improvement in Indelible Transfer Compounds, of which the following is a specification.

In many cases it is desirable that the marking transferred from a sheet of paper or other like sheet, generally known as a "pattern sheet," onto a textile fabric or the like shall be indelible, and a transfer compound of a character which when transferred onto a fabric or the like forms a permanent marking which will not be removed upon the washing of the said fabric has been sought in the past by many investigators and inventors, but for one reason or another the efforts to produce such a compound have not met with success.

The present invention has for its object generally to provide a compound which is adapted to be printed upon a sheet of paper or other suitable material either in the form of letters, numerals, words, or designs, and to be thereafter transferred from such sheet to a fabric or other like material and after transfer to remain permanently thereon as an indelible marking.

A further object of the invention is to provide an indelible transfer compound including a solid artificial resin, which is non-saponifiable and preferably of a character such that it will not melt or fuse at the ordinary temperature of boiling water (100° centigrade), whereby after such compound has been printed upon a sheet of paper or the like and transferred in known manner to a sheet of textile fabric or the like it becomes and constitutes a permanent marking therefor which cannot be removed by the washing of the fabric with soap or other ordinary detergent.

I shall not at this time undertake to refer to and point out all of the various objects and advantages of the invention but will proceed at once with a detailed description thereof from which the many advantages and purposes of the invention will be pointed out or will be apparent therefrom.

In the carrying out of my invention I obtain a good quality of commercial indelible printers' ink of which the kind employed by collar and shirt manufacturers in the mark-

ing of their products may be mentioned as types, and laundry inks and combine the same with a suitable quantity of an artificial resin which is non-saponifiable. These inks include a suitable carbon black, or may include any other suitable pigment of the desired color, combined with a carrier, such as thickened linseed oil or "varnish." This compound, as is well known, is more or less viscous, the viscosity being obtained by subjecting the linseed oil, in case that oil should be used, to slight warming or heating for a period of time. If a color other than black is desired some one of the known pigments of fast color, other than carbon, in a finely divided state may be employed.

The said resin should be non-saponifiable because if the transfer medium employed should be readily saponifiable it is found that after the goods, such as a textile fabric, have been marked therewith in the manner heretofore indicated and the material so marked washed with soap or the like saponification takes place, the character of the marking compound is thereby changed and, it is found, may be largely removed from the fabric. This would be a serious defect or objection in the case of fabrics which are to be laundered at intervals.

It is preferable also that the resin employed in combination with the ink shall be of such character that it will not melt except at a temperature above that of the boiling point of water. However, I have obtained very good results by the employment of an artificial resin of the character hereinbefore indicated, the boiling point of which was less than that of the temperature of boiling water. It must be understood, therefore, that my invention is not limited to the use of a resin having a fusing or melting point above that of the boiling point of water, but such medium may be fusible or may melt at a temperature considerably below that of the boiling point of water and on the other hand may be of a character to melt or fuse at a temperature considerably above that of the boiling point of water and still operate successfully and fairly satisfactorily.

As an example of a form or type of resin which may be used I may mention coumarone resin, with which I have achieved excellent results. For the most part the

coumarone resin heretofore employed by me has been of a character such that it would fuse or melt at a temperature above that of the boiling point of water, but as already 5 indicated I have obtained fairly satisfactory results by the use or employment of a grade of that material which fused or melted at a considerably lower temperature.

In the preparation of a compound embodying my invention the transfer medium, such as coumarone resin possessing the qualities and characteristics above indicated, is first melted or fused, after which the ink, also of the character above indicated 10 and mentioned, is introduced into the molten mass. Preferably the ink is previously warmed or heated to a point sufficient to render it sufficiently fluid and mobile to pour readily. The ink and the transfer 15 medium are employed in the proportions of one to two parts, respectively, by weight. After the transfer medium has been melted or fused the ink is poured into and thoroughly mixed with the same while in a hot 20 state.

Instead of employing ink as above described I may combine a suitable pigment, such as carbon black, yellow lakes, etc., directly with the transfer medium of the 25 character above indicated. In the preparation of the transfer compound in which the pigment is mixed directly with the coumarone resin the latter is melted and the pigment in finely powdered form and in the proper proportions is introduced into the 30 molten mass and thoroughly intermixed and mingled therewith.

In the use of the compound after the same 35 has been thoroughly mixed and intermingled in any of the ways above indicated, it is maintained at a temperature sufficient to render the same sufficiently fluid to enable its application to a printing block, cylinder or the like having thereon the letters, symbols or designs which it is desired shall be 40 placed upon the pattern sheets. By bringing the printing block, cylinder or the like into contact with these pattern sheets the letters, designs, etc. are printed thereon and after having been so printed may be transferred to a sheet of textile material or other 45 suitable material in known manner by the placing of the pattern sheet face down upon the object to which the letters, designs, etc. are to be applied, after which a hot iron 50 is applied to the reverse side of the pattern sheet. The application of a hot iron effects fusion and transfer of the compound from the pattern sheet to the sheet of textile 55 or other material.

I have also discovered that a compound embodying my invention may be produced in powdered or finely granulated form and that when so produced it is applied to the pattern sheet in a manner different from

that hereinbefore described. In case it is desired to reduce the compound to a powder before its application to the pattern sheet I employ the ingredients in different proportions than heretofore mentioned. The 60 indelible ink or printers' ink and the transfer medium are employed in the proportions of one to three parts, respectively, by weight. The proper amount of the transfer medium is heated so as to melt or fuse 65 the same and the ink is then introduced and thoroughly mixed therewith, having been first slightly warmed so as to render the same sufficiently fluid and mobile to flow readily into the molten medium. The combined mass is then allowed to cool, and is then passed through a comminuting and grinding apparatus and thereby converted 70 into a granular or powdered state. Preferably the granulated material is passed 75 through sieves in order to obtain the powder as fine as may be desired.

In the application of the powdered transfer medium to the transfer sheets the letters, symbols or designs are printed on such sheets 80 by means of an indelible or printers' ink of the character above indicated and while the letters, symbols or designs as printed upon such sheets are still moist the powdered material is sprinkled thereover 85 and a portion thereof adheres to the moist letters, symbols or designs. The material which does not adhere to these moist letters, symbols or designs is removed from the 90 sheets, after which the sheets are passed 95 underneath a flame which plays upon the sheets and upon the said letters, symbols or designs, whereby the powdered compound 100 is melted or fused and coalesces and combines with the ink previously printed or placed thereon. The letters, symbols or designs may thereafter be transferred from the transfer sheets to sheets of fabric or other material in the manner as hereinbefore described.

I have discovered that by the employment 105 of a transfer medium of the character indicated as an ingredient of a transfer compound the same is rendered indelible and may be employed as permanent markings 110 for handkerchiefs, gloves, and wearing apparel of all kinds and that when such articles have been marked with a compound embodying my invention the markings remain thereon permanently and are not removed as the result of the laundering thereof. In fact, articles marked with a compound embodying my invention have withstood the severest tests and it has been found 115 impractical or impossible to remove the markings without the employment of strong 120 alkalies, etc.

The term "pigment" employed herein and in the claims is intended to include not only carbon but also other color materials.

Having thus described my invention, what I claim and desire to secure by Letters Patent is:

1. A transfer ink for producing permanent or indelible markings on fabrics or the like, comprising an artificial resin, which is non-saponifiable, and an ink which is in itself indelible.
2. A transfer ink for producing indelible markings on fabrics and the like, comprising an artificial resin, which is non-saponifiable and fuses about or above 100° centigrade, and an ink which is in itself indelible.
3. A transfer ink in powdered form for

producing permanent or indelible markings 15 on fabrics or the like comprising, an artificial resin which is nonsaponifiable and an ink which is in itself indelible.

4. A transfer ink in powdered form for producing indelible markings on fabrics or 20 the like, comprising an artificial resin which is non-saponifiable and fuses about 100° centigrade and an ink which is in itself indelible.

In testimony that I claim the foregoing as my invention, I have hereunto signed my 25 name this 12th day of July, 1923.

HELENA S. SADTLER.